# EUROPEAN PATENT SPECIFICATION

(11) **EP 0 229 325 B1**
(45) Date of publication and mention of the grant of the patent: **04.01.1995**
(21) Application number: 86117233.6
(22) Date of filing: 11.10.1982
(51) Int. Cl.: C23C 8/80, C23C 8/26, C23C 8/32

(54) **Method of manufacturing a corrosion resistant steel component**
Verfahren zur Herstellung korrosionsbeständiger Werkstücke aus Stahl
Procédé de fabrication de pièces d'acier résistant à la corrosion

(30) Priority: 15.10.1981 GB 8131133; 18.12.1981 GB 8138318; 26.02.1982 GB 8205999; 15.07.1982 GB 8220495
(43) Date of publication of application: 22.07.1987
(62) Divisional of application: 82305400.2
(73) Proprietor: LUCAS INDUSTRIES public limited company, Birmingham, B19 2XF West Midlands (GB)
(72) Inventor: Dawes, Cyril, Sutton Coldfield West Midlands (GB); Smith, John David, West Midlands (GB)
(74) Representative: Pearce, Anthony Richmond

(56) References cited:
- EP-A- 0 061 272
- DD-A- 119 822
- DE-A- 2 715 745
- DE-B- 1 179 969
- FR-A- 1 157 201
- GB-A- 693 715
- US-A- 2 343 418
- PATENT ABSTRACTS OF JAPAN, vol. 5, no. 120 (C-65)[792], 4th August 1981;& JP-A-56 58 963 (KIYOICHI OGAWA) 22-05-1981
- PATENT ABSTRACTS OF JAPAN, vol. 4, no. 186 (C-36)[668], 20th December 1980;& JP-A-55 125 267 (KAWASAKI JUKOGYO K.K.) 26-09-1980
- CHEMICAL ABSTRACTS, vol. 84, no. 1976, page 254, abstract no. 139334q,Columbus, Ohio, US; & JP-A-75 79 441 (NIHON PARKERIZING CO., LTD) 27-06-1975
- CHEMICAL ABSTRACTS, vol. 89, no. 20, November 1978, page 254, abstract no.167562j, Columbus, Ohio, US; &JP-A-78 39 227 (NIPPON TELEGRAPH AND TELEPHONE PUBLIC CORP.) 11-04-1978

## Description

This invention relates to a method of manufacturing a corrosion resistant steel component.

It is known to improve the corrosion resistance of steel components by heat treating such components by two successive molten salt bath treatments. The first salt bath heat treatment is effected for about 2 hours at 580°C in a potassium cyanide/potassium cyanate bath. The second heat treatment is effected by quenching the components at 400°C for about 10 minutes in a second salt bath containing sodium hydroxide, potassium hydroxide, and sodium nitrate. This is followed by water quenching of the component. If it is important to restore the oxidized surface of the product to its original finish, it may be necessary to effect a lapping operation at this stage followed by re-treatment in the oxidizing bath for 20 minutes at about 400°C again followed by water quenching.

The above process suffers from a number of disadvantages which are as follows:-
1. Toxic chemicals are used which present environmental hazards.
2. In order to oxidize the toxic cyanide salt carried over from the initial hardening treatment to produce a relatively harmless carbonate salt, a double oxidation route is necessary.
3. Water quenching after the oxidizing treatments is essential to ensure removal of the salts carried over from the treatment. This in turn leads to further effluent disposal problems.

JP-A-48-75433 discloses a method of anti-corrosion surface treatment of steel where the steel is heat treated in a nitriding gaseous atmosphere in a furnace to produce an epsilon iron nitride or carbonitride surface layer thereon, and is then removed from the furnace and held in air whilst still hot for 60 to 120 seconds to produce a 2-3µm Fe₃O₄ layer. The component may be allowed to cool in air or it may be cooled by immersion in oil after the Fe₃O₄ layer has been formed.

GB-A-693715 discloses a process for finishing low carbon steel articles where the articles are heated in a case-hardening furnace to form a hardened surface thereon, quenched, drawn to reduce the surface hardness somewhat, and then tumbled until a polished surface is obtained.

It is an object of the present invention to obviate or mitigate at least some of the earlier described disadvantages.

According to the present invention, there is provided a method of manufacturing a corrosion resistant non-alloy steel component comprising the steps of heat treating a non-alloy steel component in a nitriding gaseous atmosphere to produce an epsilon iron nitride or iron carbonitride surface layer thereon; and subsequently oxidising the component to provide an oxide-rich surface layer, characterized in that between the heat treating and oxidising steps the component is cooled and mechanically surface finished.

Preferred embodiments of the invention are defined in the dependent claims 2 to 9.

With regard to the step of heat treating the component in a nitriding gaseous atmosphere to form the epsilon iron nitride or iron carbonitride surface layer, this step is typically effected at a temperature in the range of 550 to 720°C for up to 4 hours in an atmosphere of ammonia, ammonia and endothermic gas, ammonia and exothermic gas or ammonia and nitrogen, with the optional inclusion of at least one or carbon dioxide, carbon monoxide, air, water vapour and methane. The terms "exothermic gas" and "endothermic gas" are well understood in the art. Carbon dioxide, carbon monoxide, air, water vapour and exothermic gas are oxidising gases. Carbon dioxide, methane and endothermic gas are carburizing gases. It is preferred to effect the heat treatment operation so that the epsilon iron nitride surface layer has a thickness of about 25 micrometres. Thicknesses greater than about 25 micrometre can lead to exfoliation or cracking of the surface layer. Typically, such a layer thickness of about 25 micrometres can be obtained by heat treatment at 660°C for 45 minutes. Such a layer thickness may also be produced by heat treatment of 570°C for 3 hours or at 610°C for 90 minutes. However, the heat treatment temperatures and times may be employed to produce layer thicknesses less than 25 micrometres, e.g. down to 15 micrometres. For example, heat treatment of 570°C for 2 hours can be employed to produce a layer thickness of 16 to 20 micrometres.

Components produced by the method of the present invention have a fine surface finish without the need to have a wax protection system to give a good corrosion resistance. For example to produce a damper rod or a piston rod, which is often hard chromium plated, the component, after being heat treated in the nitriding gaseous atmosphere, is cooled in any desired medium, and then subjected to a lapping or other mechanical surface finishing process to a surface roughness of, for example, not more than 0.2 micrometres Rₐ. This lapping or polishing process will remove any oxide film which may have formed on the component, depending upon the medium used for cooling. After the lapping or polishing process, the component can then be oxidised at a temperature of 300 to 600°C. The actual temperature depends upon the appearance required of the steel component and, more importantly, upon the properties thereof. If the component is a component such as a damper rod which is not required to have very high fatigue properties, then the oxidising heat treatment is preferably effected at 350 to 450°C for about 15 to 5 minutes depending upon the temperature in unstripped exothermic gas. However, for good fatigue properties, the component is preferably heat treated at 500 to 600°C, more preferably, 550 to 600°C followed by quenching to retain nitrogen in solid solution in the ferritic matrix of the steel microstructure. Instead of using unstripped exothermic gas, another type of oxidising atmosphere may be employed such as steam, air or other mixture of oxygen and nitrogen, carbon dioxide and nitrogen, or carbon dioxide alone or any mixture of these gases.

Quenching is preferably effected into an oil/water emulsion. In the case of components which have been oxidised and then quenched into an oil/water emulsion, an aesthetically pleasing black finish is obtained. Quenching the component directly into an oil/water emulsion without the intermediate oxidation step does not give a black finish but a grey finish where the oxide layer is only 0.1 micrometres thick. However, quenching an already oxidised component into the oil/water emulsion does increase the degree of oxidation to a small extent and thereby darkens the colour.

During quenching in the oil/water emulsion, an atmosphere of steam is produced as a small pocket around the component within the emulsion to give a controlled cooling rate. This will give a distortion-free component with maximum properties (e.g. a component less than 1.5 milli-metre thick can have a yield strength of up to 800MPa).

Quenching into the oil/water emulsion after oxidation produces a black surface with extremely good corrosion resistance and, by virtue of the residual oily film, improved bearing properties, if these are required. In a particular embodiment, a steel component, after having had an epsilon iron nitride surface layer formed thereon by heat treatment at 570°C for about 2 hours in an atmosphere 50% ammonia and 50% endothermic gas mixture is exposed to ambient air for two seconds to effect surface oxidation and then immersed in a bath of an oil-in-water emulsion which, in this embodiment, is produced by mixing a soluble oil sold under the trade mark EVCOQUENCH GW with water in an oil:water volume ratio of 1:6. Since the component being quenched is at a temperature greater than 550°C, the resultant product has a good fatigue strength and yield strength in addition to having an aesthetically pleasing black surface with extremely good resistance to corrosion and good bearing properties in view of the absorption of oil into the surface.

Components produced in accordance with the invention which have been cooled after exposure to the nitriding atmosphere, polished and then oxidised are more economical to manufacture than hard chromium plating which also suffers from the disadvantage of creating effluent disposal problems. Additionally the gaseous treatment is cheaper than the above-mentioned salt bath treatment, particularly since the latter requires the double oxidising step.

Non-alloy steel components produced according to the present invention have a hard wear resistant layer and a surface having an extremely good resistance to humidity and salt spray corrosion. Such components also have a low coefficient of friction (similar to polished hard chromium plating) so that they are capable of being used in sliding applications. Further, such components possess a high surface tension which gives extremely low wettability which is of great help in a resisting humidity and salt spray corrosion attack and also have a pleasing aesthetic appearance (gloss blue/black according to the temperature employed in the oxidising treatment). Additionally, steel components which have been quenched from 550°C to keep nitrogen in solid solution also have good fatigue and yield strength properties.

The method of the invention has the advantage that, being of an all gaseous nature, the effluent problems associated with the salt bath heat treatment process are avoided.

The method of the invention can be performed by processors with modern gaseous atmosphere heat treatment plant without the requirement for further capital investment in plating or salt bath equipment.

We have found that the mechanism of oxygen introduction upon oxidation in the gaseous state in accordance with the invention is by way of displacement of nitrogen not merely by way of absorption of oxygen.

It will be appreciated from the previous discussion relating to the atmospheres which can be used during heat treatment of the component in a nitriding gaseous atmosphere, that, in some embodiments, the layer which is formed on the steel component would more accurately be described as being epsilon iron carbonitride layer rather than an epsilon iron nitride layer. Thus, the term "epsilon iron nitride layer" should be interpreted accordingly in this description.

The fact that the mechanism of oxygen introduction upon oxidation is by way of displacement of nitrogen rather than merely by absorption of oxygen is surprising because the resultant component has a surface finish which is visually similar to the surface finish of the known salt bath heat treated and oxidised component discussed previously. Such a salt bath heat treated and oxidised component is disclosed in "A New Approach to Salt Bath Nitrocarburising" by I.V. Etchells (Heat Treatment of Metals, 1981.4, pages 85-88) as having high contents of both oxygen and nitrogen in the component down to a depth of some 2.5 micrometres from the surface or the component. Below this, the oxygen content falls rapidly whilst the nitrogen content only falls relatively slowly. It would therefore be reasonable to have concluded that a similar structure is obtained by the process of the present invention. However, this is not the case as noted above.

In a preferred example of the invention, the surface layer portion is substantially free of nitrogen atoms.

Preferably, the surface layer portion wherein substantially all of the nitrogen atoms have been displaced by oxygen atoms extends for a depth of at least 0.2, more preferably at least 0.3, micrometre.

The resistance of the oxidised surface to corrosion is explained by the predominance of iron oxide, mainly in the form of Fe₃0₄ down to a depth of at least 0.1 micrometre and sometimes down to more than 1 micrometre in depth. However, to avoid oxide exfoliation, it is preferred for iron oxide to be present down to a depth not exceeding 1 micrometre.

In one embodiment, the surface layer portion has a composition approaching that of Fe₃0₄ in the part of the surface layer portion immediately under the surface whilst, as the depth increases, the composition has an increasing Fe0 content. Such a surface layer can be produced by exposing the component having the epsilon iron nitride layer thereon to air before quenching in water/oil emulsion.

In another embodiment, the part of the surface layer portion immediately below the surface has a composition approaching that of Fe₂0₃ but, as the depth increases, the composition becomes progresssively closer to that of Fe₃0₄. Such composition can be produced by allowing the component having the epsilon iron nitride layer thereon to cool completely in air
Attention is drawn to the disclosure in a Paper entitled "Reappraisal of Nitrocarburising and Nitriding when Applied to Design and Manufacture of Non-alloy Steel Automobile Components" by C. Dawes, D.F. Tranter, and C.G.Smith presented during a symposium entitled "Heat Treatment '79' organised by The Metals Society and American Society for Metals in Birmingham on 22nd to 24th May 1979. In this paper, there is disclosure of a non-alloy steel treated by a gaseous phase process to produce an epsilon surface layer. "Air cooling" of the material subsequent to gaseous heat treatment is mentioned in such Paper. However, this is not to be construed as meaning cooling in air, ie an oxidising atmosphere. The term "air cooling" was used as a term of art to mean slow cooling and to distinguish the cooling process from oil quenching which is a fast cooling process. In fact, the "air cooling" is more accurately described as "gas cooling" since cooling was effected in the same gaseous nitriding atmosphere used during the heat treatment step to produce the epsilon layer. It is to be noted that the Paper states that all the experiments were conducted in a small, sealed quench furnace. In a sealed quench furnace, cooling is effected in a chamber which is connected with the furnace chamber and contained in the same enclosure as the furnace chamber so that ingress of air into both chambers is prevented. In the case of the cooling referred to as "air cooling" in the Paper, the samples were merely allowed to remain in the furnace to cool naturally without being quenched in the quenching oil. That cooling in air did not take place can also be deduced from Figure 2 in the Paper where the nitrogen content remains at a level consistent with epsilon iron nitride. Further indication of the the true meaning of "air cooling" as used in the aforementioned Paper is given under the heading "Corrosion Resistance" where it is made clear that the term "air cooling" means no oil protection rather than the actual use of air to effect cooling.

In the accompanying drawings:-
Figs. 1 to 4 are graphs plotting the iron and nitrogen, iron and oxygen, or iron, oxygen and nitrogen content in a layer region of samples of steel component against depth or distance from the surface of the component, and
Fig 5 is a chart showing the effect of oxidation time in air on depth of oxide coating.

To demonstrate the effects obtained by various processing steps used in the method of the present invention, four mild steel test panels (low carbon (0.10%) steel to British Standard BS970 045 M10)approximately 25mm square and 0.55 mm thick were heat treated for two hours at 570°C in an atmosphere of 50% ammonia and 50% endothermic gas mixture (carbon monoxide, carbon dioxide, nitrogen and hydrogen). After heat treatment, the four test panels were cooled in different ways.
Sample 1 was taken straight from the heat treatment zone and, whilst in the same heat treatment atmosphere, was immediately quenched in a water-free quenching oil sold by British Petroleum under the designation QUENDILLA WA 22. This operation was effected in a sealed quench furnace.
Sample 2 was removed from the furnace, exposed to air at 20°C for 5 seconds and then quenched in an oil-in-water emulsion produced by mixing a soluble oil sold under the Trade Mark EVOCQUENCH GW with water in an oil:water volume ratio of 1:5.5.
Sample 3 was cooled by removing it from the heat treatment furnace, exposing it to air at 20°C for 1 second and then quenching it into an oil-in-water emulsion produced by mixing a soluble oil sold under the Trade Mark ILOTEMP 4 at an oil:water volume ratio of 1:10.
Sample 4 was removed from the furnace and merely allowed to cool completely in air at 20°C.

After cooling the samples were analysed as described below and the results obtained given in Tables 1 to 6 below.

The oil quenched samples were first vapour degreased and then all the test pieces were introduced into an Auger Electron Spectrometer which was evacuated down to a pressure of 1 x 10⁻⁸ torr and allowed to remain under this reduced pressure overnight to remove any gases which had been absorbed into the surface of the samples.

All four samples were then analyzed for the existence of all elements except hydrogen and helium and measured to the nearest 0.1 atomic percent of a mono layer. In the Auger Electron Spectrometer, the background vacuum was 1 x 10⁻⁸ torr, the electron beam energy was 1 - 3 KeV, the beam current was 1 microampere and the energy range was 20 - 1700 eV. A layer-by-layer analysis was conducted by using the Auger Electron Spectrometer in conjunction with sequential ion beam sputtering to remove the layers. In the ion beam sputtering technique, argon ions were used at an energy of 3 keV and a current density of 75 and 150 microampere.cm² under a gas pressure of 5 x 10⁻⁵ torr. The results of such analyses are given in Tables 1 to 4 below. Additionally, samples 1 and 3, in areas remote from the ion beam sputter damage, were then subjected to ball cratering using a 30mm diameter steel ball and a 1 miro-metre diamond paste as the polising medium. The Auger Electron Spectrometer was then used to make line scans across the crater diameters and the elemental composition on these lines was measured at a number of depths between 2 x 10⁻⁶ metres and 22 x 10⁻⁶ metres.

The elemental compositions were initially read in atomic percentages and were then calculated as weight percentages and displayed in the Tables below.

The percentages by weight of all detectable elements present in amounts greater than 0.1% were recorded.

**TABLE 1**

| Sample 1. | Composition (wt%) | | | | | | |
|---|---|---|---|---|---|---|---|
| Element | Fe | C | N | O | S | Cl | Ca |
| Depth (10⁻⁹m) | | | | | | | |
| 0 | 42.3 | 29.3 | 5.2 | 13.9 | 3.6 | 4.7 | 1.1 |
| 16 | 85.7 | 1.5 | 10.1 | 1.0 | 1.0 | 0.2 | 0.5 |
| 140 | 89.4 | 0.8 | 9.1 | 0.4 | 0.2 | 0 | 0 |
| 300 | 90.0 | 0.9 | 8.4 | 0.5 | 0.2 | 0 | 0 |
| 350 | 91.0 | 0.8 | 7.6 | 0.4 | 0.2 | 0 | 0 |

**TABLE 2**

| Sample 2 | Composition (wt%) | | | | | | | |
|---|---|---|---|---|---|---|---|---|
| Element | Fe | C | N | O | S | Cl | K | Na |
| Depth (10⁻⁹m) | | | | | | | | |
| 0 | 38.6 | 23.9 | 1.0 | 21.1 | 5.4 | 0.9 | 2.0 | 7.0 |
| 16 | 72.6 | 1.0 | 0 | 25.3 | 0.5 | 0 | 0.6 | 0 |
| 140 | 75.0 | 0.5 | 0 | 24.5 | 0 | 0 | 0 | 0 |
| 300 | 76.2 | 0.3 | 0 | 23.4 | 0 | 0 | 0 | 0 |

**TABLE 3**

| Sample 3 | Composition (wt%) | | | | | |
|---|---|---|---|---|---|---|
| Element | Fe | C | N | O | S | Cl |
| Depth (10⁻⁹m) | | | | | | |
| 0 | 57.0 | 8.9 | 0 | 31.6 | 0.7 | 1.8 |
| 16 | 72.7 | 0.3 | 0 | 27.0 | 0 | 0 |
| 140 | 74.8 | 0.2 | 0.7 | 24.3 | 0 | 0 |
| 300 | 82.7 | 0.3 | 5.1 | 12.0 | 0 | 0 |
| 430 | 83.8 | 0.3 | 6.2 | 9.8 | 0 | 0 |
| 620 | 85.6 | 0.3 | 7.4 | 6.6 | 0 | 0 |

**TABLE 4**

| Sample 4 | Composition (wt%) | | | | | | | |
|---|---|---|---|---|---|---|---|---|
| Element | Fe | C | N | O | S | Cl | K | Na |
| Depth (10⁻⁹m) | | | | | | | | |
| 0 | 46.7 | 5.0 | 1.1 | 32.9 | 0.8 | 8.7 | 3.6. | 1.1 |
| 16 | 70.5 | 0.3 | 0 | 28.8 | 0 | 0 | 0.4 | 0 |
| 140 | 73.0 | 0.1 | 0 | 26.8 | 0 | 0 | 0 | 0 |
| 300 | 73.1 | 0 | 0 | 26.9 | 0 | 0 | 0 | 0 |

**TABLE 5**

| Sample 1 (Ball Crater) | Composition (wt%) | | | |
|---|---|---|---|---|
| Element | Fe | C | N | 0 |
| Depth 10-⁶m) | | | | |
| 3.9 | 90.2 | 0.6 | 8.9 | 0.3 |
| 7.4 | 91.2 | 0.5 | 8.1 | 0.19 |
| 10.7 | 91.4 | 0.3 | 8.1 | 0.3 |
| 15.0 | 91.9 | 0.4 | 7.6 | 0.16 |
| 21.7 | 92.0 | 0.5 | 7.4 | 0.16 |

**TABLE 6**

| Sample 3 (Ball Crater) | Composition (wt%) | | | |
|---|---|---|---|---|
| Element | Fe | C | N | 0 |
| Depth (10.-6m) | | | | |
| 2.3 | 86.8 | 0.4 | 7.4 | 5.5 |
| 4.2 | 91.0 | 0.3 | 8.4 | 0.4 |
| 6.2 | 91.1 | 0.4 | 8.2 | 0.3 |
| 9.5 | 91.6 | 0.4 | 7.9 | 0.2 |
| 11.2 | 91.5 | 0.5 | 7.9 | 0.2 |

Additionally, a more detailed measurement of the variations in the elemental composition of the layers was carried out on a new area of sample 3 in the first few microns. The results obtained are shown in Table 7 below:

**TABLE 7**

| Sample 3 | Composition (wt%) | | | | |
|---|---|---|---|---|---|
| Element | Fe | C | N | O | S |
| Depth (10⁻⁶m) | | | | | |
| 0.3 | 83.0 | 0.4 | 5.0 | 11.4 | 0.2 |
| 0.4 | 84.1 | 0.5 | 5.2 | 10.3 | 0 |
| 0.6 | 85.0 | 0.3 | 5.7 | 9.0 | 0 |
| 0.9 | 86.4 | 0.3 | 6.3 | 7.0 | 0 |
| 1.3 | 85.9 | 0.3 | 6.9 | 6.9 | 0 |
| 1.6 | 86.3 | 0.14 | 6.6 | 6.9 | 0 |
| 2.3 | 87.3 | 0.2 | 5.8 | 6.6 | 0 |
| 2.9 | 88.9 | 0.2 | 6.0 | 4.9 | 0 |
| 3.9 | 90.6 | 0.4 | 6.1 | 2.9 | 0 |
| 4.9 | 92.1 | 0 | 6.6 | 1.3 | 0 |

When considering the above Tables, it is to be appreciated that the heat treatment process to which the samples were subjected is one which produces an epsilon iron carbonitride layer to a depth well in excess of 20 micrometres. The epsilon iron carbonitride layer consists of a porous and a non-porous region, the porous region extending from the surface of the sample downwardly to a depth of about 10 micrometres, and the non-porous region underlying this At a depth of 20 micrometres, the epsilon iron carbonitride layer has a typical elemental composition of 92% by weight of iron, 7.4% by weight of nitrogen, 0.4% by weight of carbon and 0.2% by weight of oxygen.

In the case of Sample 1, the elemental composition for the whole layer is consistent with the epsilon iron carbonitride region of the ternary iron-carbon-nitrogen system defined by Naumann and Langescheid (Eisenhüttenwesen 1965, 36,677). The layer of Sample 1 is also consistent with the idealized iron nitride formula Fe₂N₁₋ₓ where x is 0 to 1, for the epsilon phase reported by Lightfoot and Jack in "Kinetics of Nitriding With and Without White Layer Formation" (Proceedings of Heat Treatment Conference 1973 organised by Heat Treatment and Joint Committee of the Iron and Steel Institute), the nitrogen content being between 7.5 and 11% by weight.

In order to present the information more clearly, reference is drawn to attached Figures 1 to 4 which are graphs plotting the iron and nitrogen, iron and oxygen, or iron, oxygen and nitrogen contents in a layer region of Samples 1 to 4 respectively. The layer region chosen is one which extends from 16 x 10⁻⁹ metres to about 400 x 10⁻⁹ metres from the surface. The first measurement plotted on the graph is that at 16 x 10⁻⁹ metres, the samples having been subjected to an initial ion sputtering technique to remove foreign contaminants from the outer surface.

As can be seen from the above Tables and Figures, oxidation of the Samples after heat treatment either solely in air or initially in air and followed by quenching in the oil/water emulsion results in displacement of nitrogen by oxygen. Displacement of nitrogen is total in the outermost surface layers portions (i.e. down to a depth which may vary between 0.1 micrometre and 1 micrometre,) depending upon the time of exposure to air while the sample is hot before quenching, and also on the cooling rate in the quench. Partial displacement of the nitrogen continues in some instances to depths in excess of 1 micrometre.

Samples 2 and 3 were corrosion resistant becauseof the predominance of iron oxide mainly in the form of Fe₃0₄ to depth of at least 0.1 micrometre and sometimes down to more than 1 micrometre in depth.

In Sample 4, the iron to oxygen ratio at the extreme surface indicates a composition approaching that of Fe₂0₃ but as the depth increases into the layer, the composition becomes progressively closer to that of Fe₃0₄.

In Samples 2 and 3, the iron to oxygen ratio suggests a structure close to Fe₃0₄ in the outer surface layer portions but increasing in Fe0 on progression inwards.

It will be appreciated from comparison of Tables 2 and 3 and Figs 2 and 3 that the control of the time in air at the pre-quench temperature and also the cooling speed in the quench medium is extremely critical with respect to displacement of nitrogen from the outer surface layer portions.

Lastly, it will be apparent from an examination of the Tables and Figures that the oxygen actually displaces nitrogen from the lattice, in some cases totally and in other cases to a lesser extent but still to an extent of about 90% removal down to a depth of about 0.15 micrometre This is in direct contrast to the reported effects obained by salt bath oxidation following salt bath nitriding where oxygen is reported as being simply absorbed into the nitride lattice.

With reference to Fig. 5, the first four blocks relate to exposure of nitrocarburised component at above 550°C to air for the specified time, followed by quenching in a water/oil emulsion. The last block relates to quenching of a nitrocarburized component directly into oil without exposure to air.

Steel components according to the present invention have a corrosion resistance which is superior even to components surface treated to produce an epsilon iron nitride surface layer, oil quenched, degreased (or slow cooled under a protective atmosphere) and then dipped in a de-watering oil so that the de-watering oil is absorbed into an absorbent outer portion of the epsilon iron nitride surface layer. Table 8 below compares the corrosion resistant properties of various types of steel component:-

**TABLE 8**

| SAMPLE NO | SALT SPRAY RESISTANCE (HOURS) |
|---|---|
| 1 | 0 |
| 2 | 17 |
| 3 | 96 |
| 4 | 150+ |

The salt spray resistance was evaluated in a salt spray test in accordance with ATSM Standard B117-64 in which the component is exposed in a salt spray chamber maintained at 95+2-3°F to a salt spray prepared by dissolving 5+/- 1 parts by weight of salt in 95 parts of distilled water and adjusting the pH of the solution such that, when atomised at 95°F, the collect solution has a pH in range of 6.5 to 7.2 After removal from the salt spray test, the components are washed under running water, dried and the incidence of red rusting is assessed. Components exhibiting any red rusting are deemed to have failed.

In the above Table 8, the samples are identified as follows:-
Sample 1 = a plain, ie untreated steel component.
Sample 2 = a steel component having an epsilon iron nitride surface layer produced by the first-mentioned heat treating step in the method of the invention, followed by oil quenching and degreasing (or slow cooling under a protective atmosphere).
Sample 3 = the steel component of Sample 2 additionally dipped in a de-watering oil.
Sample 4 = the steel component having an epsilon iron nitride layer and an oxide-rich surface layer produced in accordance with the present invention after lapping the surface to a finish of 0.2 micrometres.
It is to be noted that, in the case of Sample 4, the actual salt spray resistance figure depends upon the surface finish. In a particular example, the steel component treated is a shock absorber Piston rod with a final surface finish of 0.13 to 0.15 micrometres Ra. Such a component was found to have a salt spray resistance of 250 hours.
The improvement in fatigue properties will become apparent from an examination of Table 9 below:-

**TABLE 9**

| SAMPLE | ENDURANCE LIMIT AT 10⁷ Cycles N/mm² | |
|---|---|---|
| | Plain | Notched |
| 5 | 250 | 190 |
| 6 | 440 | 350 |
| 7 | 260 | 195 |
| 8 | 435 | 345 |

The fatigue property was evaluated using an NPL-type two point loading rotary beam machine employing standard 0.30" (7.6mm) diameter NPL test pieces.
In Table 9 above:-
Sample 5 = an untreated steel component.
Sample 6 = a steel component which has an epsilon iron nitride surface layer formed thereon by heat treatment at 570°C for about 2 hours in an atmosphere of 50% ammonia and 50% endothermic gas mixture, followed by oil quenching.
Sample 7 = a steel component having an epsilon iron nitride layer produced as in Sample 6 above, and subsequently oxidised in a sodium/potassium hydroxide/sodium nitrate salt bath mixture (sold as "Degussa ABl salt") at a temperature of 400°C as recommended by the suppliers of the salt mixture.
Sample 8 = a steel component having an epsilon iron nitride surface layer formed by heat treatment as in Sample 6 but subsequently oxidised in steam at 540°C for 30 minutes, followed by oil quenching.

It will be seen that oxidation using the salt bath treatment as per Sample 7 above reduces the fatigue properties almost back to the level of Sample 5. This is caused by nitrogen being precipitated from solid solution. The gaseous oxidation technique as per Sample 8 can be applied over a much wider temperature range. Consequently by using a controlled oxidation process at 550°C followed by oil quenching, the improved fatigue properties associated with the heat treatment process as per Sample 6 are maintained.

This occurs because at the higher temperature, most of the nitrogen remains in solid solution and is maintained therein by the subsequent oil quenching.

A specific example of the present invention will now be described:-
A shock absorber piston rod having a length of 230mm, a diameter of 12.5 mm, and an initial surface roughness of 0.13 to 0.15 micrometres Ra was manufactured by machining a bar of low carbon steel (BS970-045M10) and was heat treated for two hours at 570°C in an atmosphere of 50% ammonia and 50% endothermic gas mixture (Carbon monoxide, carbon dioxide, nitrogen and hydrogen). The rod was then cooled slowly under the protection of the same atmosphere as used in the above mentioned heat treatment. The resultant rod had a 20 micrometre thick layer of epsilon iron nitride thereon and a surface roughness of 0.64 micrometres Ra.

In view of the high surface finish requirements for the piston rod, it was lapped at this stage to a surface roughness of 0.13 micrometres Ra.

Following this, the rod was oxidised in an exothermic gas mixture containing its moisture of combustion for 10 minutes at 400°C to produce a 0.5 micrometre thick oxide-rich surface layer. The piston rod was then cooled by water quenching.

The piston rod was found to have a salt spray resistance of 250 hours according to the above described salt spray test.

In a modification of the above described specific example, the rod was oxidised for 15 minutes at 400°C in the exothermic gas mixture, but during the last 5 minutes of the 15 minute cycle, sulphur dioxide was introduced into the furnace in an amount such as to give a concentration of 0.25% by volume in the furnace atmosphere. Such a technique caused about 1% of the iron oxide (Fe₂0₃) on the surface of the rod to be converted to iron sulphide which gave an aesthetically pleasing shiny black surface to the rod.

The technique of sulphiding is not restricted to components in the form of damper rods and can be used in respect of any components on which it is desirable to have a black hard-wearing surface. With surface finishes greater than 0.25 micrometres Ra, it will be necessary to wax coat in order to produce the desired corrosion resistance. To effect sulphiding, the S0₂ content in the oxidizing furnace may be up to 1% by volume and the temperature may be in the range of 300°C to 600°C. The S0₂ will normally be added to the furnace at some stage after the oxidizing heat treatment has started in order to convert some of the already formed iron oxide to iron sulphide.

The invention is particularly applicable to non-alloy steels having a low carbon content, for example up to 0.5% carbon.

## Claims

1. A method of manufacturing a manufacturing a corrosion resistant non-alloy steel component comprising the steps of heat treating a non-alloy steel component in a nitriding gaseous atmosphere to produce an epsilon iron nitride or iron carbonitride surface layer thereon; and subsequently oxidising the component to provide an oxide-rich surface layer, characterized in that between the heat treating and oxidising steps the component is cooled and mechanically surface finished.

2. A method as claimed in Claim 1, wherein the mechanical surface finishing is effected so that the surface roughness of the component does not exceed 0.2 micrometres Rₐ.

3. A method as claimed in Claim 1 or 2, wherein the oxidising is effected by heat treating the surface finished component in a gaseous atmosphere at 300 to 600°C.

4. A method as claimed in Claim 3, wherein the component is a piston rod.

5. A method as claimed in Claim 4, wherein the oxidising is effected by heat treating the component in an exothermic gas mixture containing its moisture of combustion.

6. A method as claimed in Claim 5, wherein the oxide-rich surface layer is 0.5 micrometre thick and is Fe₃O₄.

7. A method as claimed in Claim 4, wherein the surface finishing step is effected so that the component after the oxidising step has a final surface finish of 0.13 to 0.15 micrometre Rₐ.

8. A method as claimed in any one of Claims 1 to 7, wherein the heat treatment in the nitriding gaseous atmosphere is effected at a temperature of 550 to 720°C.

9. A method as claimed in any one of Claims 1 to 7, wherein a sulphur-containing compound is introduced into the oxidising atmosphere to produce iron sulphide whereby the surface of the component contains iron sulphide as well as iron oxide.

## Patentansprüche

1. Verfahren zur Herstellung eines korrosionsbeständigen Nichtlegierungsstahl-Bauteils, das die Schritte der Wärmebehandlung eines Nichtlegierungsstahl-Bauteils in einer nitrierenden Gasatmosphäre, um eine Epsilon-Eisennitrid- oder Eisencarbonitridschicht darauf zu erzeugen, und der anschließenden Oxidation des Bauteils vorsieht, um eine oxidreiche Oberflächenschicht vorzusehen,
dadurch gekennzeichnet,
daß das Bauteil zwischen den Wärmebehandlungs- und Oxidationsschritten abgekühlt und mechanisch oberflächenendbearbeitet wird.

2. Verfahren nach Anspruch 1,
bei dem die mechanische Oberflächenendbearbeitung so erfolgt, daß die Oberflächenrauhigkeit des Bauteils 0,2 µm Rₐ nicht übersteigt.

3. Verfahren nach Anspruch 1 oder 2,
bei dem die Oxidation durch Wärmebehandlung des oberflächenendbearbeiteten Bauteils in einer Gasatmosphäre bei 300 bis 600 °C erfolgt.

4. Verfahren nach Anspruch 3,
bei dem das Bauteil eine Kolbenstange ist.

5. Verfahren nach Anspruch 4,
bei dem die Oxidation durch Wärmebehandlung des Bauteils in einer ihre Verbrennungsfeuchtigkeit enthaltenden exothermen Gasmischung erfolgt.

6. Verfahren nach Anspruch 5,
bei dem die oxidreiche Oberflächenschicht 0,5 µm dick ist und Fe₃O₄ ist.

7. Verfahren nach Anspruch 4,
bei dem der Oberflächenendbearbeitungsschritt so durchgeführt wird, daß das Bauteil nach dem Oxidationsschritt einen Endoberflächenzustand von 0,13 bis 0,15 µm Rₐ hat.

8. Verfahren nach irgendeinem der Ansprüche 1 bis 7,
bei dem die Wärmebehandlung in der nitrierenden Gasatmosphäre bei einer Temperatur von 550 bis 720 °C erfolgt.

9. Verfahren nach irgendeinem der Ansprüche 1 bis 7,
bei dem eine schwefelhaltige Verbindung in die oxidierende Atmosphäre zur Erzeugung von Eisensulfid eingeführt wird, wodurch die Oberfläche des Bauteils Eisensulfid sowie Eisenoxid enthält.

## Revendications

1. Procédé de fabrication d'un élément en acier non allié résistant à la corrosion, comprenant les étapes de traitement thermique d'un élément en acier non allié dans une atmosphère gazeuse de nitruration pour produire sur celui-ci une couche superficielle d'epsilon nitrure de fer ou de carbonitrure de fer ; et d'oxydation subséquente de l'élément pour fournir une couche superficielle riche en oxyde, caractérisé en ce qu'entre les étapes de traitement thermique et d'oxydation, l'élément est refroidi et sa surface est finie de façon mécanique.

2. Procédé selon la revendication 1, dans lequel la finition superficielle mécanique est effectuée de sorte que la rugosité superficielle de l'élément ne dépasse pas 0,2 µm Rₐ.

3. Procédé selon la revendication 1 ou 2, dans lequel l'oxydation est effectuée en traitant thermiquement l'élément fini en surface dans une atmosphère gazeuse de 300 à 600 °C.

4. Procédé selon la revendication 3, dans lequel l'élément est une tige de piston.

5. Procédé selon la revendication 4, dans lequel l'oxydation est effectuée en traitant thermiquement l'élément dans un mélange de gaz exothermique contenant l'humidité de sa combustion.

6. Procédé selon la revendication 5, dans lequel la couche superficielle riche en oxyde présente une épaisseur de 0,5 µm et est constituée par le Fe3O4.

7. Procédé selon la revendication 4, dans lequel l'étape de finition superficielle est effectuée de sorte que l'élément, après l'étape d'oxydation, ait une surface de finition de 0,13 à 0,15 µm Rₐ.

8. Procédé selon l'une quelconque des revendications 1 à 7, dans lequel le traitement thermique dans l'atmosphère gazeuse de nitruration est effectué à la température de 550 à 720 °C.

9. Procédé selon l'une quelconque des revendications 1 à 7, dans lequel un composé contenant du soufre est introduit dans l'atmosphère oxydante pour produire du sulfure de fer, de sorte que la surface de l'élément contienne du sulfure de fer ainsi que de l'oxyde de fer.
